

1

2,810,733

**PERACID EPOXIDATION OF FATTY ACID ESTERS**

Frank P. Greenspan, Buffalo, N. Y., assignor, by mesne assignments, to Food Machinery and Chemical Corporation, San Jose, Calif., a corporation of Delaware

No Drawing. Application March 23, 1954,  
Serial No. 418,208

10 Claims. (Cl. 260—348.5)

This application pertains to a novel type of epoxidized triglycerides and more particularly to a method of partially epoxidizing triglycerides such as occur in unsaturated oils.

Methods for epoxidizing unsaturated oils by means of an organic peracid have been described previously. In these methods the ethylenic unsaturated material is treated with a quantity of organic peracid sufficient to epoxidize substantially all double bonds present in the material. In other words, previously published epoxidation methods, starting out with an oil possessing a certain degree of ethylenic unsaturation, were performed in such a way as to result in a fully epoxidized oil possessing essentially no ethylenic unsaturation. Such fully epoxidized oils were found to be suitable as plasticizers for polymeric substances, such as polyvinyl chloride, either as such or in form of their derivatives.

Because unepoxidized oils, possessing original unsaturation, are not compatible with plastics which it is desired to plasticize, previous epoxidation methods all aimed at complete epoxidation so as to leave only a marginal amount of unsaturation. I have now found that under certain conditions, oils which have not been fully epoxidized are not only compatible with plastics but actually have better performance characteristics than fully epoxidized oils. However, such partially epoxidized oils cannot be produced by arbitrarily restricting the extent of epoxidation, but have to be produced by a strictly controlled epoxidation process. Such partially epoxidized oils furthermore require in their manufacture, reduced amounts of epoxidizing agent, such as peracid or hydrogen peroxide, because obviously partial epoxidation of a given quantity of a given oil requires less reactants than complete epoxidation. Thus partially epoxidized oils prepared in accordance with this invention have been found to be not only better in performance but also cheaper to manufacture than fully epoxidized oils. Moreover, these novel partially epoxidized oils have various useful properties of interest in the manufacture of intermediate detergents, lubricant additives, etc.

I have now found that such partially epoxidized oils can be produced by a critically modified epoxidation process. In epoxidation methods designed to produce fully epoxidized oils, the amount of peracid used is calculated on the amount of ethylenic unsaturation present in the oil. That is to say, that ordinarily at least 1 mole of peracid or hydrogen peroxide is employed for each double bond in each mole of the unsaturated fatty acid chains in the oil. Thus sufficient peracid is available to transform substantially all double bonds present into the corresponding epoxy groups. Such epoxidation reactions may be carried out with prepared organic peracids such as peracetic acid, performic acid, perbutyric acid and others. These reactions may also be carried out using the so-called "in situ" method, wherein peracid is formed during the course of the reaction in the reaction medium from calculated quantities of hydrogen peroxide and the corresponding organic acid. Furthermore, such epoxidation reactions, using prepared peracids or peracids formed in situ, may be carried out with or without a solvent present in the reaction mixture, which solvents may be benzene, hexane or other inert solvents.

In contrast to epoxidation methods resulting in complete epoxidation, the present invention pertains to a method resulting in a controlled and defined partial epoxidation. Here epoxidation is carried out in such a manner that substantially all of the ethylenic unsaturation in those chains of the oil that are mono-unsaturated fatty acid chains is epoxidized but only one double bond epoxidized in those chains that are poly-unsaturated fatty acid chains. There results a defined epoxy compound containing saturated fatty acid chains, saturated epoxy fatty acid chains and unsaturated epoxy fatty acid chains. This controlled epoxidation method and the resulting products are, therefore, distinct and different from methods which arbitrarily restrict degree epoxidation and produce a random distribution of epoxy groups and double bonds. Taking into account total unsaturation; that is total number of double bonds in a naturally occurring oil and taking into account the approximate per cent fatty acid composition of such oils, it becomes possible to calculate the amount of peracid required to produce a defined degree of partial epoxidation.

The amount of peracid required for such partial epoxidation will, of course, vary with the unsaturated oil to be treated because the composition of such oils; that is, their content of mono-ethylenic unsaturated higher fatty acid, di-ethylenic unsaturated higher fatty acid and poly-ethylenic unsaturated higher fatty acid varies. Corn oil, for instance, contains essentially only mono-and di-unsaturated acids aside from some saturated acids. Linseed oil, on the other hand, contains mono-, di-, and tri-ethylenic unsaturated fatty acids, together with some saturated acids. As pointed out above, this composition of the oil, as well as the respective percentages of mono-, di-, and poly-ethylenic unsaturated acids have to be taken into account when calculating the amount of peracid required for defined partial epoxidation.

In any case of partial epoxidation of a naturally occurring oil, the reaction has to be carried out in such a manner that substantially all double bonds in the mono-unsaturated fatty acids present are epoxidized and, therefore, disappear. However, the multiple double bonds in the double unsaturated and polyunsaturated fatty acids present, substantially one double bond only in each fatty acid chain should be epoxidized. Therefore, the proper amount of peracid is calculated in every case so as to epoxidize all of the mono-unsaturated radicals and one double bond of the poly-unsaturates. Knowing the composition of a given natural oil, calculation of the proper amount of peracid, sufficient to give the desired percentage of reacted double bonds, is possible. Per cent double bonds reacted can also be expressed and checked by calculating the iodine number to be expected for a certain degree of partial epoxidation.

The proper amount of peracid required for partial epoxidation in accordance with this invention is calculated on a molar basis and corresponds to 1-1.3 mole of peracid for each double bond in each mole of mono-unsaturated esterified acid and 1-1.3 mole of peroxide for one double bond in each mole of polyunsaturated esterified acid.

An example for calculating the required amount of peracid may be given for the case of partial epoxidation of linseed oil. A typical commercial linseed oil will contain about 19% oleic acid containing 1 double bond in the chain, 24% linoleic acid containing 2 double bonds in the chain and 47% linolenic acid containing 3 double bonds in the chain. The equivalent of the total number

of double bonds in a single average fatty acid chain of the triglyceride can then be arrived at as follows:

19.0% oleic acid with 1 double bond equivalent to 0.190  
 24.1% linoleic acid with 2 double bonds equivalent to 0.482  
 47.4% linolenic acid with 3 double bonds equivalent to 1.422  
 Total number of double bonds equivalent to 2.094

In the controlled partial epoxidation of linseed oil all of the double bonds of the oleic acid chains, one of the 2 double bonds in the linoleic acid chains and one of the 3 double bonds in the linolenic acid chains are to be epoxidized. Therefore, the equivalent to the number of double bonds to be reacted can be represented as follows:

19.0% oleic acid with 1 double bond equivalent to 0.190  
 24.1% linoleic acid with 1 double bond equivalent to 0.241  
 47.4% linolenic acid with 1 double bond equivalent to 0.474  
 Total number of double bonds to be reacted equivalent to 0.905

The percent double bonds to be theoretically reacted in linseed oil is then

$$\frac{0.905}{2.094} \times 100 = 43.3\%$$

On this basis the theoretical amount of epoxidation reagent required can be calculated. 1000 gram linseed oil with an iodine number of 171 corresponds to 6.74 mole of ethylenic unsaturation and to epoxidize 43.37 thereof requires 43.3% of 6.74 mole or 2.91 mole of reagent.

The percent double bonds to be reacted can be calculated in the same way for other oils, whereby the following percent figures are obtained:

|               | Percent |
|---------------|---------|
| Corn oil      | 68.0    |
| Menhaden oil  | 33.2    |
| Safflower oil | 55.0    |
| Soybean oil   | 57.7    |

This sample calculation will suffice to indicate how the proper amount of peracid is to be calculated for different natural oils and for different peracids. The following examples, although not restrictive, are intended to show partial epoxidation procedures for different naturally occurring unsaturated oils, different peracids as epoxidizing agents and different epoxidation techniques. Sample techniques are described for the use of prepared peracids, for use of "in situ" techniques and, furthermore, with and without the use of a solvent. It should be pointed out that in all cases, substantially quantitative yields of the desired partially epoxidized oil were obtained in relatively very short reaction times and in a highly economical way. The various oils were subjected to controlled partial epoxidation; that is, epoxidation was carried up to a percentage lower than 100% epoxidation. In the following Table 1, percent epoxidation reaction is given for the different oils in the different examples. The term "percent epoxidation reaction" indicates how far the controlled partial epoxidation has been carried. Variations in the figures given for percent epoxidation are essentially due to the fact that specific oil samples will frequently show a composition different from the average composition published for such oils. Moreover, as in organic reactions generally, a certain excess of epoxidizing reagent is used in carrying out the reaction to take care of unavoidable losses and experimental errors. In general, the amount of epoxidizing agent on a mole basis is 1 to 1.3 moles per mole of desired double bond to be reacted upon.

4  
 TABLE 1

| Example | Oil       | Percent Epoxidation Reaction |
|---------|-----------|------------------------------|
| 1.      | Safflower | 63.6                         |
| 2.      | do        | 60.5                         |
| 3.      | do        | 52.5                         |
| 4.      | do        | 60.4                         |
| 5.      | do        | 60.0                         |
| 10.     | Corn      | 80.0                         |
| 7.      | Linseed   | 46.3                         |
| 8.      | Menhaden  | 42.5                         |
| 9.      | Soybean   | 64.5                         |
| 10.     | Safflower | 60.4                         |

15 Before giving the actual experimental data and figures, the general procedure will be described here. All the following experimental examples were carried out by weighing the proper amount of the oil to be treated into a three-neck flask equipped with a condenser, thermometer and stirrer. To the oil was then added the proper amount of solvent, if a solvent was used. Where prepared peracids were employed, a quantity of a buffer, such as anhydrous sodium acetate, was then added in an amount sufficient to neutralize the mineral acid catalyst used in preparing the peracid and present in the product as used. This addition was carried out slowly over a period of time while maintaining temperature between approximately 15 and 35° C. For in situ operation, no anhydrous sodium acetate need be used and the calculated amount of hydrogen peroxide and concentrated organic acid is added. In all the experiments, the temperature was kept near the upper limit of the temperature range after all reagents have been added to the reaction flask. 20 In each experiment the composition of the oil is given in terms of the constituent fatty acid.

25 The percent double bonds to be reacted can be calculated in the same way for other oils, whereby the following percent figures are obtained:

30

Percent

40

Corn oil

percent 16.4

45

Menhaden oil

do 77.7

50

Safflower oil

do 0.3

55

Soybean oil

do 6.6

60

Iodine number

140

65 700 g. of safflower oil, equivalent to 3.85 moles of ethylenic unsaturation, were reacted in presence of 23.1 g. of anhydrous sodium acetate with 2.41 mole peracetic acid (459.0 g. peracetic acid 40%). This was added over a period of 1 hour and 50 minutes at 15 to 20° C. and temperature then maintained at 20 to 30° C. for a total reaction time of 3½ hours. After washing, the product was analyzed and found to contain:

Percent epoxy 4.9  
 Iodine number 51

70 *Example 2*  
 75 700 g. of safflower oil, equivalent to 3.85 moles of ethylenic unsaturation of the same composition as used in Example 1, were reacted in presence of 23.1 g. of anhydrous sodium acetate and of 700 g. of benzene with 2.41 mole peracetic acid (459.0 g. peracetic acid 40%). This was added over a period of 1 hour and 50 minutes at 15 to 20° C. and temperature then maintained at 20 to 30° C. for a total reaction time of 3½ hours. After washing, the product was analyzed and found to contain:

Percent epoxy 4.6  
 Iodine number 53

## Example 3

1000 g. of safflower oil, equivalent to 5.5 mole of ethylenic unsaturation, of the same composition as used in Example 1, and 200 g. of benzene were put into the reaction flask. To this were added 1.67 mole acetic acid (100 g. glacial acetic) and 6.7 g. of 50% sulfuric acid. Then 3.47 mole  $H_2O_2$  (236.0 g. of 50%  $H_2O_2$ ) were added over a period of 1½ hours while maintaining the temperature of the mixture between 40° and 54° C. The reaction was continued for a total reaction time of 13 hours maintaining the temperature at 60 to 65° C. After washing, the product was analyzed and found to contain:

|                        |     |    |
|------------------------|-----|----|
| Percent oxirane oxygen | 4.1 | 15 |
| Iodine number          | 67  |    |

## Example 4

1000 g. of safflower oil, equivalent to 5.5 mole of ethylenic unsaturation, of the same composition as in Example 1, 1.67 mole acetic acid (100.0 g. glacial acetic) and 14.8 g. of 50% sulfuric acid were put in the reaction flask. Then 3.97 mole  $H_2O_2$  (270.0 g. of 50%  $H_2O_2$ ) were added over a period of 1 hour while keeping the temperature between 53 and 65° C. Total reaction time was 9 hours at a temperature of 60 to 65° C. After washing, the product was analyzed and found to contain:

|               |     |    |
|---------------|-----|----|
| Percent epoxy | 4.3 | 10 |
| Iodine number | 55  |    |

## Example 5

500 g. of safflower oil, corresponding to 2.75 mole of ethylenic unsaturation, of the same composition as used in Example 1, and 21.5 g. of anhydrous sodium acetate were placed in the reaction flask. Then 1.73 mole of perbutyric acid (430 g. of 42% perbutyric acid) were added over a period of 2 hours while maintaining the temperature at 15 to 20° C. The reaction was continued for an additional 2 hours at 30 to 35° C. to give a total reaction time of 4 hours. After washing, the product was analyzed and found to contain:

|               |     |    |
|---------------|-----|----|
| Percent epoxy | 4.4 | 20 |
| Iodine number | 56  |    |

## Example 6

## CORN OIL

|                  |         |      |
|------------------|---------|------|
| Oil composition: |         |      |
| Oleic acid       | percent | 46.3 |
| Linoleic acid    | do      | 41.7 |
| Saturated acids  | do      | 12.0 |
| Iodine number    |         | 119  |

1500 g. of corn oil, equivalent to 7.03 moles of ethylenic unsaturation, were reacted in presence of 55.0 g. of anhydrous sodium acetate with 5.27 mole of peracetic acid (1005.0 g. peracetic acid 40%). This was added over a period of 2 hours and 45 minutes at 15 to 20° C. and the temperature was then permitted to rise slowly over a total reaction time of 4 hours and 15 minutes to 55° C. After washing, the product was analyzed and found to contain:

|               |     |    |
|---------------|-----|----|
| Percent epoxy | 5.3 | 30 |
| Iodine number | 24  |    |

## Example 7

## LINSEED OIL

|                  |         |      |
|------------------|---------|------|
| Oil composition: |         |      |
| Oleic acid       | percent | 19.0 |
| Linoleic acid    | do      | 24.1 |
| Linolenic acid   | do      | 47.4 |
| Saturated acids  | do      | 9.5  |
| Iodine number    |         | 171  |

1000 g. of linseed oil, equivalent to 6.74 moles of ethylenic unsaturation, were reacted in presence of 32.0 g. of anhydrous sodium acetate with 3.34 mole peracetic acid (635.3 g. peracetic acid 40%). This was added over a period of 1 hour and 10 minutes at a temperature of 17 to 20° C. and the temperature then maintained at

17 to 33° C. for a total reaction time of 3 hours and 15 minutes. After washing, the product was analyzed and found to contain:

|               |     |   |
|---------------|-----|---|
| Percent epoxy | 4.5 | 5 |
| Iodine number | 92  |   |

Example 8  
MENHADEN OIL

|                  |         |      |
|------------------|---------|------|
| Oil composition: |         |      |
| Hendecenoic acid | percent | 15.5 |
| $C_{18}$ acids   | do      | 30.0 |
| $C_{20}$ acids   | do      | 19.0 |
| $C_{22}$ acids   | do      | 12.0 |
| Saturated acids  | do      | 23.5 |
| Iodine number    |         | 174  |

600 g. of menhaden oil, equivalent to 4.12 moles of ethylenic unsaturation, were reacted in presence of 14.3 g. of anhydrous sodium acetate with 1.50 mole of peracetic acid (285.0 g. peracetic acid 40%). This was added over a period of 1 hour and 5 minutes at about 20° C. and the temperature then maintained at 24 to 32° C. for a total reaction time of 3 hours and 45 minutes. After washing, the product was analyzed and found to contain:

|               |     |    |
|---------------|-----|----|
| Percent epoxy | 3.7 | 20 |
| Iodine number | 100 |    |

## Example 9

## SOYBEAN OIL

|                  |         |      |
|------------------|---------|------|
| Oil composition: |         |      |
| Palmitoleic acid | percent | 0.4  |
| Oleic acid       | do      | 29.7 |
| Linoleic acid    | do      | 50.4 |
| Linolenic acid   | do      | 6.5  |
| Saturated acids  | do      | 13.0 |
| Iodine number    |         | 135  |

600 g. of soybean oil, equivalent to 3.19 moles of ethylenic unsaturation, were reacted in presence of 18.3 g. of anhydrous sodium acetate with 1.92 mole of peracetic acid (365.0 g. peracetic acid 40%). This was added over a period of 1 hour and 10 minutes at 20 to 25° C. and temperature then maintained at 26 to 33° C. for a total reaction time of 3 hours and 20 minutes. After washing, the product was analyzed and found to contain:

|               |     |    |
|---------------|-----|----|
| Percent epoxy | 4.6 | 30 |
| Iodine number | 48  |    |

## Example 10

## SAFFLOWER OIL

100 g. of safflower oil, corresponding to 0.550 mole of ethylenic unsaturation, of the same composition as used in Example 1, and 0.165 mole of formic acid (8.46 g. of 90% formic acid) were placed in the reaction flask. Then 0.396 mole of  $H_2O_2$  (27.0 g. 50%  $H_2O_2$ ) were added over a 5 minute period at 26° C. and the temperature then maintained between 26 and 35° C. for an additional 22½ hours. After washing, the product was analyzed and found to contain:

|               |     |    |
|---------------|-----|----|
| Percent epoxy | 4.5 | 40 |
| Iodine number | 58  |    |

The over-all efficiency of the method of this invention is further indicated by the very high and, in some cases, theoretical yield of partially epoxidized triglyceride obtained. These yields were:

|          |  |               |
|----------|--|---------------|
| Example: |  | Yield percent |
| 1        |  | 96            |
| 2        |  | 96            |
| 3        |  | 97            |
| 4        |  | 88            |
| 5        |  | 90            |
| 6        |  | 95            |
| 7        |  | 100           |
| 8        |  | 88            |
| 9        |  | 92            |
| 10       |  | 96            |

From the foregoing description and examples it will be seen that there is outlined a method for obtaining stated partially epoxidized ethylenic unsaturated higher fatty oils in periods of time shorter than required for complete epoxidation. By limiting the amount of epoxidizing reagent to substantially that required to epoxidize the ethylenic unsaturation in a mono-unsaturated chain, and to that required to epoxidize one only of the ethylenic unsaturated positions in a polyethylenic unsaturated chain, products are produced that are found to be compatible as plasticizers in certain resin films.

Substantially complete epoxidation results at the desired positions indicated above, in shorter periods of time by reason of the greatly increased reaction time required to epoxidize the second, third, etc., of the ethylenic positions in a poly-unsaturated chain.

The epoxidizing reagent may be a lower aliphatic peracid, such as peracetic acid, or may be hydrogen peroxide and the lower aliphatic acid in the presence of from about 0.5% to 5% sulfuric acid. Where the peracid is employed, the temperature of reaction is preferably low, from about 15° C. to 35° C. and the reaction time, on the order of 1 to 4 hours. Where peroxide and lower aliphatic acid are employed, the temperature of reaction is somewhat higher and the duration of the reaction longer.

What is claimed is:

1. The method of epoxidizing unsaturated fatty acid esters contained in naturally occurring unsaturated oils which comprises heating said oils under epoxidizing conditions with a lower aliphatic peracid, the amount of which corresponds to 1 to 1.3 moles of peracid for each double bond in each mole of mono-unsaturated esterified acid plus 1 to 1.3 moles of lower aliphatic peracid for one double bond only of each mole of poly-unsaturated esterified acid.

2. The method of epoxidizing unsaturated fatty acid esters contained in naturally occurring unsaturated oils which comprises heating said oils under epoxidizing conditions with hydrogen peroxide, a lower aliphatic acid and sulfuric acid, the amount of the hydrogen peroxide corresponding to 1 to 1.3 moles, and the amount of lower aliphatic acid corresponding to about 0.25 to 1 mole for each double bond in each mole of mono-unsaturated esterified acid plus 1 to 1.3 moles of hydrogen peroxide, and the amount of sulfuric acid corresponding to about 0.5 to 5% of the total weight of lower aliphatic acid and hydrogen peroxide for one double bond only of each mole of poly-unsaturated esterified acid.

3. The method of epoxidizing unsaturated fatty acid esters contained in naturally occurring unsaturated oils which comprises heating said oils under epoxidizing conditions with peracetic acid, the amount of which corresponds to 1 to 1.3 moles of peracid for each double bond in each mole of mono-unsaturated esterified acid plus

1 to 1.3 moles of peracetic acid for one double bond only of each mole of poly-unsaturated esterified acid.

4. The method of epoxidizing unsaturated fatty acid esters contained in naturally occurring unsaturated oils which comprises heating said oils under epoxidizing conditions with performic acid, the amount of which corresponds to 1 to 1.3 moles of peracid for each double bond in each mole of mono-unsaturated esterified acid plus 1 to 1.3 moles of performic acid for one double bond only of each mole of poly-unsaturated esterified acid.

5. The method of epoxidizing unsaturated fatty acid esters contained in naturally occurring unsaturated oils which comprises heating said oils under epoxidizing conditions with perbutyric acid, the amount of which corresponds to 1 to 1.3 moles of peracid for each double bond in each mole of mono-unsaturated esterified acid plus 1 to 1.3 moles of perbutyric acid for one double bond only of each mole of poly-unsaturated esterified acid.

6. The method of epoxidizing safflower oil which comprises heating the safflower oil under epoxidizing conditions with a lower aliphatic peracid, the amount of which corresponds to about 55% of that required completely to epoxidize the oil.

7. The method of epoxidizing corn oil which comprises heating the corn oil under epoxidizing conditions with a lower aliphatic peracid, the amount of which corresponds to about 68.0% of that required completely to epoxidize the oil.

8. The method of epoxidizing menhaden oil which comprises heating the menhaden oil under epoxidizing conditions with a lower aliphatic peracid, the amount of which corresponds to about 33.2% of that required completely to epoxidize the oil.

9. The method of epoxidizing soybean oil which comprises heating the soybean oil under epoxidizing conditions with a lower aliphatic peracid, the amount of which corresponds to about 57.7% of that required completely to epoxidize the oil.

10. The method of epoxidizing linseed oil which comprises heating the linseed oil under epoxidizing conditions with a lower aliphatic peracid, the amount of which corresponds to about 43.3% of that required completely to epoxidize the oil.

#### References Cited in the file of this patent

#### UNITED STATES PATENTS

- |           |                     |       |               |
|-----------|---------------------|-------|---------------|
| 2,312,535 | Fieser              | ----- | Mar. 2, 1943  |
| 2,485,160 | Niederhauser et al. | ----- | Oct. 18, 1949 |
| 2,569,502 | Swern et al.        | ----- | Oct. 2, 1951  |

#### OTHER REFERENCES

- Findley et al.: J. Am. Chem. Soc. 67:412 (1945).  
 Ralston: "Fatty Acids and Their Derivs.", p. 414 (1948),  
 John Wiley and Sons.